

## UNITED STATES PATENT OFFICE

2,276,602

PROCESS OF DYEING AND THE PRODUCTS  
THUS OBTAINED

Jürgen von Klenck, Frankfort-on-the-Main,  
Hochst, and Josef Nüsslein, Frankfort-on-  
the-Main, Germany, assignors to General  
Aniline & Film Corporation, a corporation of  
Delaware

No Drawing. Application July 27, 1939, Serial  
No. 286,868. In Germany August 3, 1938

7 Claims. (Cl. 8—54)

The present invention relates to a process of dyeing and to the products thus obtained.

As is known fibrous material of animal origin may be dyed with acid dyestuffs, for instance dyestuffs of the anthraquinone, triphenylmethane or azo-series.

This invention is based on the observation that animal fibers and other nitrogenous substances, especially fibrous materials, may be dyed with acid compounds soluble in water, which are obtainable by condensation of plastic nitrogenous compounds, for instance compounds containing amino-groups, at an elevated temperature and in the presence of an acid-binding agent, with organic compounds containing, besides chromophoric groups, groups which render the products soluble in water, especially acid groups, and groups which can be exchanged, especially acid radicals capable of splitting off acid by reaction with the hydrogen atoms of the amino-groups of the plastic material, the latter groups being eliminated. The dyestuffs which may be used in the present process may for instance be made according to the process of application Serial No. 212,514, filed June 8, 1938, now Patent No. 2,232,892, in the name of Jürgen von Klenck for "Process of dyeing nitrogenous compounds of high molecular weight and the products thus obtained."

Besides animal fibrous materials such as wool, silk and hair, other nitrogenous compounds, for instance, gelatine, glue, casein, if desired hardened by means of formaldehyde, may be dyed by this invention; also other nitrogenous products of high molecular weight, for instance, plastic masses, such as condensation products of urea, toluene sulfamide or melamine with formaldehyde, or fibrous materials from such materials, furthermore, animalized cellulose fibers or the like.

The dyestuffs used contain besides acid groups, such as sulfo-groups or carboxyl groups, and a chromophoric radical, for instance of the anthraquinone, triphenylmethane or azo-series a nitrogenous group of high molecular weight, for instance, the residue of gelatine, casein, wool degradation products or other albuminous substances and nitrogenous plastic masses.

These dyestuffs whose shades depend upon the nature of the condensation components selected are dyed by one or other of the processes usual for dyeing with acid wool dyestuffs, for instance, in an acid or neutral bath with the aid of sodium sulfate, sodium bisulfate or ammonium sulfate. The solution obtained by the condensation may either be used after neutralization directly for dyeing or the dyestuff formed may first be isolated by evaporation or salting out and used in a fresh bath for dyeing the material. The usual adjuvants, for instance, dispersing, wetting and

levelling agents may be added to the dyeing baths.

The dyeings thus produced are distinguished by a good evenness. Their properties of fastness depend in high degree upon the nature of the components that are condensed to form the dyestuff. The fastness of the dyeings especially the fastness to wet processing may be enhanced by an after-treatment with agents which effect a polymerization, agglomeration or hardening of the nitrogenous bodies of high molecular weight which have been used in making the dyestuff, for instance, gelatine.

Suitable agents for the after-treatment are those of tanning action, such as chromium salts and formaldehyde. The after-treatment may be applied at ordinary or raised temperature on wet or dry dyeings with or without addition of a catalyst. If plastic masses capable of being hardened are used in the manufacture of the dye-stuffs, the dyeing need only be heated in order to harden it and thus to improve the fastness.

The following examples serve to illustrate the invention, but they are not intended to limit it thereto:

1. 1 gram of 1-bromo-2-anthraquinonesulfonic acid is treated with the same quantity of gelatine, 2 grams of sodium bicarbonate, 1 gram of calcined sodium carbonate and 0.1 gram of crystallized copper sulfate in 100 cc. of water at boiling temperature until the brown solution, which was at first colorless, no longer changes its color; this happens after about 3-4 hours. The solution thus obtained is neutralized.

2. A dye bath is prepared which contains

|                        |          |     |
|------------------------|----------|-----|
| Water                  | cc       | 200 |
| Sulfuric acid          | per cent | 4   |
| Sodium sulfate crystal | lb       | 10  |

calculated on the weight of the goods, and 10 cc. of the neutralized dyestuff solution. 10 grams of wool are dyed in the usual manner in this bath for 1 hour at the boil. An even dyeing of the full brown is obtained. The fastness to wet-processing may be improved by after-treating the goods with an acid solution, at raised temperature, containing 2 per cent. of formaldehyde or 1½ per cent. of potassium bichromate, calculated on the weight of the goods.

3. Instead of the condensation product from bromanthraquinonesulfonic acid and gelatine there may be used the condensation product from gelatine and 1-amino-4-iodanthraquinone-2,6-disulfonic acid (violet dyeing) or 1-chloro-4-nitro-8-anthraquinonesulfonic acid (blue dyeing) or the azo-compound from ortho-chloraniline and 1-hydroxy-4-naphthalenesulfonic acid (red dyeing).

4. 1 gram of 1,4-dichloro-6-anthraquinonesulfonic acid is treated for 4 hours at boiling tem-

perature with the same quantity of gelatine and 2 grams of sodium bicarbonate, 1 gram of calcined sodium carbonate and 0.1 gram of copper bromide in 100 cc. of water. The dark brown solution obtained is neutralized by means of an acid and the condensation product formed is precipitated by adding saturated sodium chloride solution. After filtering and drying about 1.7 grams of dyestuff are obtained.

A dyebath is prepared by means of

|                                                                          | Per cent |
|--------------------------------------------------------------------------|----------|
| Formic acid                                                              | 5        |
| Sodium sulfate crystals                                                  | 10       |
| Dyestuff                                                                 | 17       |
| Oxethylation product from oleyl alcohol and<br>20 mols of ethylene oxide | 1        |

10 grams of wool are dyed in this boiling bath for 1 hour. The wool is dyed a clear deep brown shade.

3. 1 gram of 1-amino-4-bromo-2-anthraquinone-carboxylic acid is treated with the same quantity of gelatine and 2 grams of sodium bicarbonate, 1 gram of crystallized sodium carbonate, 0.2 gram of crystallized copper sulfate and 3 cc. of pyridine in 100 cc. of hot water. The deep violet solution obtained is neutralized by means of an acid and  $\frac{1}{10}$  of the solution is used for preparing a dyebath containing

|                         | Per cent |
|-------------------------|----------|
| Sulfuric acid           | 4        |
| Sodium sulfate crystals | 10       |

10 grams of wool are dyed a deep violet shade after 1 hour's boiling in this bath.

4. 1 gram of 1-anilido-4-iodo-2-anthraquinone-sulfonic acid is treated for 2 hours with the same quantity of gelatine, 2 grams of sodium bicarbonate, 1 gram of crystallized sodium carbonate, 0.2 gram of crystallized copper sulfate, 3 cc. of pyridine and 0.1 gram of copper bromide in 100 cc. of water at boiling temperature. The deep blue solution obtained is neutralized and  $\frac{1}{10}$  of the solution is added to a dyebath prepared with 5 per cent. of acetic acid and 10 per cent. of crystallized sodium sulfate. 10 grams of wool are dyed in this bath a clear deep blue shade. The fastness of this very even dyeing may be improved by after-treatment with potassium bichromate and acetic acid, the shade assuming a somewhat greener coloration.

5. 1 gram of 1-anilido-4-iodo-2-anthraquinone-sulfonic acid is treated for 5 hours at boiling temperature with 2 grams of a water-soluble product, obtainable by condensation of urea with formaldehyde, in an aqueous solution containing

|                             | Grams |
|-----------------------------|-------|
| Sodium bicarbonate          | 2     |
| Calcined sodium carbonate   | 1     |
| Crystallized copper sulfate | 0.1   |

The deep-blue solution is treated with saturated sodium chloride solution whereupon the condensation product, a blue dyestuff, is precipitated.

A dyebath is prepared with

|                             | Per cent |
|-----------------------------|----------|
| Sulfuric acid               | 4        |
| Crystallized sodium sulfate | 10       |
| Oleic acid methyl tauride   | 0.5      |

$\frac{1}{10}$  of the blue dyestuff obtained is added. 10 grams of wool are dyed a clear vivid blue by boiling it in this bath for 1 hour. The dyeing is treated for 10 minutes at 130° C. in a drying oven whereupon its fastness to wet-processing is improved.

6. 1 gram of 1,4-dichloro-6-anthraquinonesulfonic acid, 2 grams of the urea-formaldehyde condensation product mentioned in Example 5, 2 grams of sodium bicarbonate, 1 gram of calcined sodium carbonate and 0.1 gram of copper bromide in 100 cc. of water are heated for 6 hours at boiling temperature. A brown solution is formed. After neutralization with sulfuric acid  $\frac{1}{10}$  of the solution is added to a dyebath prepared with

|                             | Per cent |
|-----------------------------|----------|
| Ammonium sulfate            | 5        |
| Crystallized sodium sulfate | 10       |

After boiling for one hour 10 grams of wool are dyed a vivid brown.

7. 1 gram of 1-bromo-2-anthraquinonesulfonic acid is treated according to Example 1 at boiling temperature with the same quantity of gelatine, 2 grams of sodium bicarbonate, 1 gram of calcined sodium carbonate and 0.1 gram of crystallized copper sulfate in 100 cc. of water, until the brown solution which was at first colorless, no longer changes its color: this happens after about 3-4 hours. The solution thus obtained is neutralized.

25 A dyebath is prepared which contains

|                         |             |
|-------------------------|-------------|
| Water                   | cc. 200     |
| Sulfuric acid           | per cent. 4 |
| Sodium sulfate crystals | do. 10      |

30 calculated on the weight of the goods—and  $\frac{1}{10}$  of the neutralized dyestuff solution obtained as described above. 10 grams of fibers produced on the basis of casein are dyed in the usual manner in this bath for 1 hour at the boil. An even dyeing of a full brown is obtained. The fastness to wet-processing may be improved essentially by after-treating the goods, at raised temperature, with an acid solution containing 2 per cent. of formaldehyde or 1½ per cent. of potassium bichromate, calculated on the weight of the goods.

35 A similar dyeing is obtained, when cuprammonium silk is dyed in the dyebath described, which has been animalized by incorporating a condensation product from chlorine-hard paraffin and ethylenediamine (cf. British Patent No. 440,647). Also this dyeing which is distinguished by a good evenness, may be improved in its fastness to wet-processing by the indicated after-treatment.

40 8. 1 gram of 1,4-dichloro-6-anthraquinonesulfonic acid is treated according to Example 2 for 4 hours at boiling temperature with the same quantity of gelatine and 2 grams of sodium bicarbonate, 1 gram of calcined sodium carbonate and 0.1 gram of copper bromide in 100 cc. of water. The dark brown solution obtained is neutralized by means of an acid and the dyestuff formed is precipitated by adding saturated sodium chloride solution. After filtering and drying about 1.7 grams of dyestuff are obtained.

45 A dyebath is prepared by means of

|                                                                          | Per cent |
|--------------------------------------------------------------------------|----------|
| Formic acid                                                              | 5        |
| Sodium sulfate crystals                                                  | 10       |
| Dyestuff                                                                 | 1.7      |
| Oxethylation product from oleyl alcohol<br>and 20 mols of ethylene oxide | 1        |

50 75 10 grams of viscose artificial silk are dyed in this bath for 1 hour at boiling temperature, which has been animalized by incorporating a condensation product from a bromide of a mixture of alcohols of high molecular weight with polymeric ethylenimine (cf. French Patent No.

810,395). The fiber is dyed a clear deep brown shade.

9. 1 gram of 1-anilido-4-iodo-2-anthraquinone-sulfonic acid is treated according to Example 4 for 2 hours with the same quantity of gelatine, 2 grams of sodium bicarbonate, 2 grams of crystallized sodium carbonate, 0.2 gram of crystallized copper sulfate, 3 cc. of pyridine and 0.1 gram of copper bromide in 100 cc. of water at boiling temperature. The deep blue solution obtained is neutralized and  $\frac{1}{2}$  of the solution is added to a dyebath prepared with 5 per cent. of acetic acid and 10 per cent. of crystallized sodium sulfate. Viscose artificial silk, which was animalized by incorporating casein, is dyed in this bath clear blue shades. The fastness of this very even dyeing may be improved essentially by after-treatment with potassium bichromate and acetic acid, the shade assuming a somewhat greener coloration.

We claim:

1. The process which comprises dyeing fibrous materials containing amino groups with acid dyestuffs obtained by reacting plastic materials containing amino groups, at an elevated temperature and in the presence of an acid-binding agent, with organic compounds containing chromophoric groups, water-solubilizing acid groups and acid radicals the acid radicals being capable of splitting off acid by reaction with the hydrogen atoms of the amino groups of the plastic material and splitting off only said acid radicals by the reaction.

2. The process which comprises dyeing fibrous materials containing amino groups with acid dyestuffs obtained by reacting plastic materials containing amino groups, at an elevated temperature and in the presence of an acid-binding agent, with  $\alpha$ -halogen-anthraquinonesulfonic acids.

3. The process which comprises dyeing fibrous materials containing amino groups with acid dyestuffs obtained by reacting gelatine, at an ele-

40 vated temperature and in the presence of an acid-binding agent, with  $\alpha$ -halogen-anthraquinonesulfonic acids.

4. The process which comprises dyeing wool with acid dyestuffs obtained by reacting plastic materials containing amino groups, at an elevated temperature and in the presence of an acid-binding agent, with  $\alpha$ -halogen-anthraquinonesulfonic acids.

5. The process which comprises dyeing wool with acid dyestuffs obtained by reacting gelatine at an elevated temperature and in the presence of an acid-binding agent, with  $\alpha$ -halogen-anthraquinonesulfonic acids.

10 6. The process which comprises dyeing fibrous materials containing amino groups with acid dyestuffs obtained by reacting plastic materials containing amino groups at an elevated temperature and in the presence of an acid-binding agent,

15 20 with organic compounds containing chromophoric groups, water-solubilizing acid groups and acid radicals the acid radicals being capable of splitting off acid by reaction with the hydrogen atoms of the amino groups of the plastic material and splitting off only said acid radicals by the reaction and after-treating the dyeings in order to enhance their fastness with agents which effect a polymerization of the plastic materials.

25 30 7. Fibrous materials containing amino groups dyed with acid dyestuffs obtained by reacting plastic materials containing amino groups at an elevated temperature and in the presence of an acid-binding agent, with organic compounds containing chromophoric groups, water-solubilizing acid groups and acid radicals the acid radicals being capable of splitting off acid by reaction with the hydrogen atoms of the amino groups of the plastic material and splitting off only said acid radicals by the reaction.

JÜRGEN V. KLENCK.  
JOSEF NÜSSLEIN.